

## UNITED STATES PATENT OFFICE

2,420,729

## DYEING WITH INDIGOID VAT DYESTUFFS

Edward Weber, Winchester, Mass., assignor to  
 Allied Chemical & Dye Corporation, New York,  
 N. Y., a corporation of New York

No Drawing. Application March 30, 1944,  
 Serial No. 528,771

12 Claims. (Cl. 8—25)

1

This invention relates to a method of dyeing piece-goods comprising animal fibers, and especially woolen piece-goods, with indigoid vat dyestuffs. It relates more particularly to an improved method for dyeing piece-goods composed of animal fibers, and especially woolen piece-goods, full shades with indigoid vat dyestuffs, and especially indigo, in an ordinary piece-dye kettle (winch or reel machine).

The dyeing of piece-goods comprising animal fibers with indigoid vat dyestuffs, and especially indigo, presents a number of difficulties which ordinarily are not encountered in the dyeing of cotton and other vegetable fibers. Thus, because of the chemical nature of the animal fibers, it is necessary to avoid the use of strongly alkaline vats. It has accordingly been the practice to dye woolen piece-goods in a weakly alkaline vat (produced by reducing the vat dyestuff with aqueous sodium hydrosulfite and a weak alkali, such as ammonium hydroxide, sodium carbonate, or the like) which preferably also contains a dispersion assistant (such as a protective colloid or an organic dispersing agent; for example, glue, gelatin, synthetic organic compounds of the alkyl aryl sulfonate type, and the like).

Further, owing to the relatively low solubility of the leuco compounds of the vat dyestuffs, in such vats, special dyeing procedures requiring the use of special apparatus have been employed heretofore in order to obtain full shades which are sufficiently even (level) and fast to crocking to be commercially acceptable.

In view of its desirable fastness properties, indigo has been employed extensively for the production of full navy blue shades on wool, especially for military and civilian uniforms. The production of full navy blue shades on woolen cloth, such as 11-ounce flannel and 16-ounce Melton, presents special difficulties owing to the fact that such woolen cloth is not easily penetrated, and indigo, when dyed from vats compatible with wool, is not very soluble in the vat, with the result that dyeings produced with sufficient indigo to give a full navy blue shade are not fast to washing, crocking and rubbing. Hence, many dyers have preferred to dye the raw woolen stock rather than the piece-goods. Others have dyed woolen piece-goods with indigo from an ammonia-hydrosulfite-glue vat by working

the cloth in the vat, below the surface of the dye liquor, in open width by hand ("hand-hawking"), or stretched upon frames or on so-called "hawking-machines."

5 Prior to the present invention, it was considered necessary to avoid any creasing, folding or wrinkling of the cloth during the sojourn of the cloth in the dyebath in order to avoid unevenness, streaking, and/or differential fastness to crocking of the finished cloth. This has restricted the dyeing of woolen piece-goods and related piece-goods comprising animal fibers to dye houses having the special equipment necessary for such open-width operations.

10 15 An object of the present invention is to provide a method for dyeing piece-goods comprising animal fibers, and especially woolen piece-goods, with indigoid vat dyestuffs from a vat in conventional piece-dyeing apparatus.

20 Another object of the present invention is to provide a method for dyeing piece-goods comprising animal fibers, and especially woolen piece-goods, with indigo from a weakly alkaline vat in conventional piece-dyeing apparatus.

25 A further object of the present invention is to provide a method for dyeing piece-goods comprising animal fibers in the rope form with indigoid vat dyestuffs in full shades having good evenness and fastness to crocking.

30 A specific object of the present invention is to provide a method for dyeing woolen piece-goods in the rope form with indigo from an ammonia-hydrosulfite vat in full shades having good evenness and fastness to crocking.

35 Other objects of the invention in part will be obvious and in part will appear hereinafter.

According to the present invention, the above objects are accomplished by dyeing piece-goods comprising animal fibers, and especially woolen piece-goods, in rope form, in a vat of an indigoid vat dyestuff, the extent of the dyeing being insufficient to produce a full shade, and bringing the dyeing to full shade by dyeing the piece-goods with a wool color. The wool color may be 40 one which dyes wool from a neutral or an acid bath or it may be a chrome color. When a chrome color is used, the dyeing treatment with the chrome color is preferably carried out by the after-chroming process.

45 50 If it is attempted to dye woolen piece-goods

full navy blue shades with indigo alone in rope form in conventional piece-dyeing equipment, such as winch or reel machines, amounts of dye-stuff are required which are so large that the dyeings rub off, are not fast to crocking, and are streaked and uneven. According to the present invention, it has been found possible to produce satisfactory full navy blue shades on woolen piece-goods by effecting the major development of the navy blue shades with a restricted amount of indigo which can be applied in conventional piece-dyeing equipment without such deleterious results, and bringing the dyeings to full shade by "filling" with wool colors. Good dyeings are obtained by using amounts ranging from about 10 to about 25 pounds of Indigo NAC 20% paste or equivalent (that is, about 2 to about 5 pounds of indigo on the dry basis) per 100 pounds of wool, and effecting the vatting with from about 1 $\frac{1}{4}$  to 4 $\frac{1}{2}$  pounds of sodium hydrosulfite and from about 1 to about 2 $\frac{1}{2}$  pounds of sodium hydroxide. The employment of materially less than 10 pounds of 20% Indigo NAC paste or equivalent per 100 pounds of wool is perfectly feasible where weaker shades than a full navy blue are desired; but for full navy blue shades such lesser amounts are undesirable, since they must be "filled" with so much chrome or other wool colors that the resultant dyeings fail to possess sufficient of the shade and other characteristics peculiar to indigo. On the other hand, it is not generally desirable to employ materially more than 25 pounds of 20% Indigo NAC paste or equivalent per 100 pounds of wool since difficulties in the complete and satisfactory application of the dyestuff to the wool result.

The dyeing with the wool color may take place prior to the dyeing with the indigoid vat dye-stuff or subsequent to the dyeing with the indigoid vat dyestuff. For the production of full shades with indigo on woolen piece-goods, the dyeing with the wool color is preferably carried out with a chrome color and prior to the dyeing with indigo (that is, by chrome color-bottoming); since it has been found that in the method of dyeing in the rope form of the present invention, the application of indigo to a bottom of chrome colors provides a more rapid method of dyeing, and leads to dyeings possessing somewhat superior fastness to rubbing and washing.

The invention will be illustrated by the following specific example, but it is to be understood that the invention is not limited to the details thereof and that changes may be made without departing from the scope of the invention.

#### EXAMPLE

Eleven-ounce woolen piece-goods were processed and dyed in rope form in an ordinary piece-dye kettle (winch machine) open to the atmosphere in the following manner, the ratio of the goods to the dyebath or liquor being always maintained at about 1:20. The amount of reagent used in each case is given in terms of 100 pounds of cloth.

#### Washing

The goods were first washed by circulating them for 30 minutes in a bath at 180° F. and composed of water, 2 lbs. of "Nacconol NR" (a commercial surface-active agent comprising a mixture of alkyl benzene sodium sulfonates derived from kerosene) and 4 lbs. of 26% ammonium hydroxide. The goods were then washed free from alkali with water.

#### Bottoming with chrome dyes

A dyebath was prepared by warming the water in the kettle to 110° F. and adding:

- 5 2 oz. of Alizarol Azurine ECA  
3 lbs. 8 oz. of Superchrome Blue BC  
1 lb. 3 oz. of Superchrome Blue B High Conc. (C. I. 202)  
2 lbs. 8 oz. of Superchrome Red ECB  
10 3 oz. of Superchrome Yellow RN (C. I. 197)  
10 lbs. of calcined Glauber's salt (Na<sub>2</sub>SO<sub>4</sub>)  
6 lbs. of 56% acetic acid.

The winch was set in motion, and the dyebath was heated to boiling during one hour. The bath 15 was boiled for an additional hour and then cooled to 160° F. (by displacing part of the exhausted dyebath with cold water) at which point 3 lbs. of sodium bichromate, dissolved in water, were introduced. The bath was reheated to boiling 20 during 15 minutes, and boiled for 45 minutes, after which it was displaced with water. The goods were rinsed until a clear rinse liquor was obtained.

#### Topping with indigo

- 25 25 A stock vat of indigo was prepared by pasting 10 lbs. of Indigo NAC 20% paste (Color Index 1177) with a solution of 1 lb. of caustic soda flakes in 5 lbs. of cold water, sprinkling in 1 lb. 30 11 oz. of sodium hydrosulfite powder, and heating the resulting mixture to 125° F. until reduction of the indigo to the leuco compound was complete.

A bath was prepared by adding to the water 35 in the kettle:

- 35 6 lbs. of 26% ammonium hydroxide, 2 lbs. of animal glue, and 3 lbs. of sodium hydrosulfite. The resulting mixture was heated to 125° F. and the goods were circulated for 10 minutes. The stock vat of indigo was quickly added to the 40 bath, and dyeing was carried out at 125° F. for 20 minutes. Then 10 lbs. of calcined Glauber's salt (Na<sub>2</sub>SO<sub>4</sub>), dissolved in 100 lbs. of water, were added slowly during 10 minutes to exhaust the 45 dyebath. The goods were then rinsed and circulated through cold running water until the leuco-indigo was oxidized substantially complete.

The dyed goods thus obtained were scoured 50 with soap in the conventional manner to remove loosely-held indigo, rinsed and dried.

The goods were dyed full and well-penetrated navy blue shades possessing good evenness (levelness) and fastness to crocking.

55 The temperature of the dyebath is preferably maintained at about 120° to about 130° F. as is usual in dyeing wool with an ammoniacal indigo vat, but other temperatures can be employed.

The exhaustion of the ammoniacal indigo vat 60 (dyebath) is effected with sodium sulfate in the above example. While this results in improved tinctorial strength of the dyeings, as disclosed and claimed in my application Serial No. 528,772, filed March 30, 1944, it may be accomplished 65 according to methods well known in the art, for example, by adding various acidic substances (e. g., acids or acid salts; such as, ammonium sulfate, bisulfate, formate, acetate, chloride, etc.).

While in the above example woolen piece-goods 70 are dyed first with a chrome color, followed by after-chroming, and then with indigo from an ammonia-hydrosulfite-glue vat, the invention is not limited thereto.

Thus, the invention includes the dyeing of 75 piece-goods comprising proteinous fibers of vari-

ous kinds, including natural animal fibers (such as wool, silk, hair and the like) and artificial animal fibers (such as those derived from casein, soybean and the like), all of which are comprehended within the generic term "animal fibers" herein and in the claims.

Further, other vat dyestuffs of the indigoid series may be similarly employed instead of indigo; as for example:

Vat Orange R—Color Index No. 1217.

Vat Red Violet RH—Color Index No. 1212.

Vat Pink FF—Am. Assoc. Textile Chemists and Colorists, Vol. XIX (1942), page 523.

Brilliant Indigo 4BR—Color Index No. 1184.

Brilliant Indigo KMR—Color Index No. 1183.

The indigo or other indigoid vat dyestuff may be applied from an ammonia-hydrosulfite-glue vat of the type employed in the above example or from other vats suitable for the dyeing of animal fibers with indigoid vat dyestuffs, a number of which are known. Thus, the vat may contain a leuco compound of the vat dyestuff, a hydrosulfite and a non-caustic alkali (e. g., sodium carbonate, an ethanolamine, ethylene diamine, disodium phosphate, etc.). In dyeing woolen piece-goods with indigo in accordance with the present invention, ammonium hydroxide is preferably employed inasmuch as other non-caustic alkalies lead to somewhat weaker dyes. Preferably the vat also contains a dispersion assistant, which may be animal glue or another dispersion assistant, a number of which are mentioned above.

The invention also includes the application of a wool color, as a topping color, to a fabric dyed with an indigoid vat dyestuff. The wool color may be a neutral wool dye, an acid wool dye or a chrome color. When a chrome color is used, the chrome treatment may be carried out in any of the usual ways for the dyeing of animal fibers with chrome colors. As above noted, in the preferred practice of the present invention, the goods are given a preliminary dyeing with a chrome color and are then dyed with the indigoid vat dyestuff.

The relative amounts of indigoid vat dyestuff and wool color necessary for the production of a particular shade can be readily determined by simple test dyeings. Thus, a test dyeing of a sample of woolen cloth may be carried out with the indigoid vat dyestuff in an amount less than sufficient to produce the particular shade, and the necessary amount of wool color to bring the resulting dyeing to full shade may then be determined by dyeing the resulting sample of indigoid dyed goods with the selected wool color.

I claim:

1. A method of producing full shades with an indigoid vat dyestuff on piece-goods comprising animal fibers which comprises dyeing the piece-goods in rope form in a vat of an indigoid vat dyestuff, the extent of the dyeing being less than sufficient to produce a full shade, and dyeing the piece-goods with a wool color to a sufficient extent to produce a full shade with the dyeing of the indigoid vat dyestuff.

2. The method of dyeing piece-goods comprising animal fibers claimed in claim 1, wherein the dyeing with the wool color precedes the dyeing with the indigoid vat dyestuff.

3. A method of producing full shades with indigo on piece-goods comprising animal fibers which comprises dyeing the piece-goods in rope form in an indigo vat, the extent of the dyeing

being less than sufficient to produce a full shade, and dyeing the piece-goods with a wool color to a sufficient extent to produce a full shade with the indigo dyeing.

4. The method of dyeing piece-goods comprising animal fibers claimed in claim 3, wherein the dyeing with the wool color precedes the dyeing with indigo and the wool color is a chrome color.

5. A method of producing full shades with an indigoid vat dyestuff on woolen piece-goods which comprises dyeing the woolen piece-goods in rope form in a vat of an indigoid vat dyestuff, the extent of the dyeing being less than sufficient to produce a full shade, and dyeing the woolen piece-goods with a wool color to a sufficient extent to produce a full shade with the dyeing of the indigoid vat dyestuff.

6. The method of dyeing piece-goods comprising animal fibers claimed in claim 5, wherein the dyeing with the wool color precedes the dyeing with the indigoid vat dyestuff.

7. A method of producing full shades with an indigold vat dyestuff on woolen piece-goods which comprises dyeing the woolen piece-goods in an acid dyebath containing a chrome color, after-chroming the dyeing, and dyeing the resulting woolen piece-goods in rope form in a vat containing an indigold vat dyestuff in leuco form, a hydrosulfite, ammonium hydroxide and an organic dispersions assistant, the extent of the dyeing with the indigold vat dyestuff being less than sufficient to produce a full shade.

8. A method of producing full shades with indigo on woolen piece-goods which comprises dyeing woolen piece-goods in rope form with indigo from a weakly alkaline vat and with a wool color, the extent of the dyeing with indigo being less than sufficient to produce a full shade.

9. A method of producing full shades with indigo on woolen piece-goods which comprises dyeing woolen piece-goods in rope form with indigo from an ammonia-hydrosulfite-glue vat, and with a chrome color followed by after-chroming, the extent of the dyeing with indigo being less than sufficient to produce a full shade.

10. The method of dyeing woolen piece-goods in full navy blue shades which comprises dyeing woolen piece-goods with a wool color, rinsing the resulting dyed goods, working the resulting goods in rope form in an ammonia-hydrosulfite indigo vat, and oxidizing leuco-indigo on the goods to indigo, the amount of indigo employed being about 2 pounds to about 5 pounds, on the dry basis, per hundred pounds of wool.

11. The method of dyeing woolen piece-goods in full navy blue shades which comprises working woolen piece-goods in an acid dyebath containing a chrome color, after-chroming the dyed goods, rinsing the chromed goods, working the resulting goods in rope form in an ammonia-hydrosulfite indigo vat, and oxidizing leuco-indigo on the goods to indigo, the amount of indigo employed being about 2 pounds to about 5 pounds, on the dry basis, per hundred pounds of wool.

12. The method of dyeing woolen piece-goods in full navy blue shades which comprises working woolen piece-goods in rope form in an acid dyebath containing a chrome color, acetic acid and sodium sulfate, after-chroming the dyed goods with the addition of sodium bichromate to the dyebath, rinsing the chromed goods, working the resulting goods in rope form in an ammonia-hydrosulfite-glue indigo vat, and oxidizing leuco-indigo on the goods to indigo, the amount of indigo employed being about 2 pounds to about

5 pounds, on the dry basis, per hundred pounds of wool.

EDWARD WEBER.

REFERENCES CITED

The following references are of record in the file of this patent:

UNITED STATES PATENTS

| Number    | Name     | Date           | 10 |
|-----------|----------|----------------|----|
| 1,148,966 | Hebden   | Aug. 3, 1915   |    |
| 1,199,273 | Iljinsky | Sept. 26, 1916 |    |
| 443,026   | Weiss    | Dec. 16, 1890  |    |
| 129,753   | Scala    | July 23, 1872  |    |

| Number    | Name     | Date          |
|-----------|----------|---------------|
| 794,050   | Sellet   | July 4, 1905  |
| 1,682,453 | Willheim | Aug. 28, 1928 |

FOREIGN PATENTS

| Number  | Country       | Date          |
|---------|---------------|---------------|
| 213,266 | Great Britain | Jan. 1, 1925  |
| 84,974  | Germany       | Jan. 15, 1896 |
| 379,321 | Great Britain | Aug. 23, 1932 |
| 669,189 | France        | July 27, 1929 |

OTHER REFERENCES

Whittaker: Dyeing with Coal Tar Dyestuffs, 2nd ed., 1926, pp. 129, 130, 131, 140, 141.